

# UNITED STATES PATENT OFFICE.

JOSEPH M. BROWN, OF AUSTIN, ARKANSAS.

## TANNING PROCESS.

1,323,956.

Specification of Letters Patent.

Patented Dec. 2, 1919.

No Drawing.

Application filed April 4, 1919. Serial No. 287,449.

*To all whom it may concern:*

Be it known that I, JOSEPH M. BROWN, a citizen of the United States, residing at Austin, in the county of Lonoke and State of 5 Arkansas, have invented a new and useful Tanning Process, of which the following is a specification.

This invention relates to a process of tanning hides.

10 The objects of the invention are to provide a tanning process which is suitable for all grades of leather, which is quick and sure in its results, yet not expensive, which produces a leather of great durability, high 15 finish and desirable color and as nearly waterproof as possible, and which may be carried out by a person unskilled in the art of tanning so as to produce a uniform product.

To attain these objects, I follow the process now to be described.

First the dry hide is soaked in water until perfectly soft and well washed; then the loose fat or flesh is removed. The hide must now undergo depilation or unhairing, which 25 is accomplished by using a concentrated lime solution. Into enough water to cover the hide, sufficient slaked lime is put to form a thin batter. When this is cool, the hide is dipped three or four times to make sure the lime reaches every part of it; then is placed 30 in the batter and allowed to remain until the hair slips easily. A period of 24 to 48 hours is usually sufficient.

The action of the lime on the hide is 35 marked, causing it to become plump and swollen and at the same time loosening the hair so that on scraping with a blunt knife the hair comes off readily. The lime also gives to the hide a greater firmness, which is 40 very desirable in the subsequent operations.

When the hair slips, the hide is raised out of the solution, placed on a smooth hard surface and unhaired. The lime must now be removed because it would interfere with the 45 tanning if retained. To accomplish this, the hide is preferably put in running water for 24 to 48 hours, though still water may be used if it is changed three or four times daily. When the hide feels soft and rough 50 to the hand which is passed over the grain side, the lime has been removed. The hide is now ready for tanning.

Into enough water to cover the hide I dissolve cutch in the proportion of 1 pound 55 of cutch to 10 pounds of green hide. The solution is preferably mixed in a tin or gal-

vanized vessel and strained into a wooden vat or tub. When the cutch solution is tepid or not unbearably hot to the hand, the hide is dipped into it. The dipping is repeated 60 three or four times at intervals of 5 or 10 minutes to set the grain and secure a uniform color.

To the solution is now added a quantity of powdered white vitriol (zinc sulfate). One-half as much zinc sulfate is used as cutch, that is one-half pound to every 10 pounds of green hide. The skin is left in the bath until thoroughly tanned. This condition may be ascertained by finding when the hide becomes 70 a uniform color throughout its greatest thickness.

The hide should now be taken out of the solution and rinsed in clear water. This done, it should be spread out on a smooth surface 75 and oiled on both sides with a mixture of neat's foot oil and fish oil or else common tanner's oil. The hide is left in this position until the oil has struck in and the hide is almost dry; then the wrinkles are ironed out 80 of the grain side of the leather by one of the implements customarily used for this purpose and the flesh side is smoothed with sand paper or equivalent means. The leather is now ready for the market.

When making sole leather, the above method is followed except that the oil is applied lightly on the grain side only.

When tanning all large hides, weighing as much as 15 pounds or more green, only one-half the required amount of cutch and white vitriol is used when the hides are put for the first time in the tanning bath. On the second day, the hides should be taken out and repelted; then the solution is strengthened 95 with the undissolved portion of the chemicals, and the hides returned.

The above-described process produces a leather which is durable and has a high finish, besides being as nearly waterproof as it 100 is possible to make leather. The process itself is simple, requires no great skill or special apparatus, and has the further virtue of being rapid. The cutch is an active tanning agent, while the white vitriol aids greatly 105 in producing a firm, tough leather, especially desirable for harness or sole purposes.

Having described my invention what is claimed is:—

1. That method of tanning which consists in dipping a hide into a bath at successive intervals, said bath consisting of a solu-

tion of cutch in water, adding white vitriol to the bath, and leaving the hide therein until completely tanned.

2. That method of tanning which consists  
5 in taking a quantity of water sufficient to  
cover a hide, dissolving cutch in the water in  
the proportion of one pound of cutch to ten  
pounds of hide, dipping the hide into said  
solution at successive intervals, adding to  
10 the solution powdered white vitriol of one-  
half the weight of the cutch, and returning

the hide to the solution until completely  
tanned.

In testimony, that I claim the foregoing  
as my own, I have hereto affixed my signature  
in the presence of two witnesses. 15

<sup>his</sup>  
JOSEPH M. X BROWN.  
mark

Witnesses:

BRICKELLE DAVIS,  
HAGAN SHIVE.